

## UNITED STATES PATENT OFFICE

2,202,041

PROCESS FOR OBTAINING CREPE EFFECTS  
ON FABRICS

Hans Altwegg, Paris, France, and Armin Eichler,  
Freiburg in Breisgau, Germany, assignors to  
E. I. du Pont de Nemours & Company, a cor-  
poration of Delaware

No Drawing. Original application April 6, 1931,  
Serial No. 528,240. Divided and this applica-  
tion October 2, 1937, Serial No. 166,984. In  
Germany April 11, 1930

2 Claims. (Cl. 28—1)

Crepe effects are generally obtained on mate-  
rials by the use of highly twisted warp or weft  
threads and special effects are obtained by defi-  
nite alternation of warp or weft yarns, highly  
5 twisted to left and to right. This process can be  
applied to artificial silks which, like viscose silks,  
for example, consist of regenerated cellulose.

Fabrics which contain as their warp or weft  
highly twisted viscose yarns show a valuable crepe  
10 effect on being treated with warm water, that is,  
for example, after having been subjected to a  
process for removing the dressing or to a dyeing  
process. This results from the fact that highly  
twisted viscose yarns possess the property, on be-  
15 ing treated with water or with aqueous solutions  
of all kinds, of curling and simultaneously shrink-  
ing on drying. If such yarns are present as warp  
or weft in the fabric and if these fabrics are  
treated in the way indicated, distortion of the  
20 fabric takes place resulting in the so-called crepe  
effect.

However, if this method of treatment is applied  
to fabrics, the warp or weft of which consists  
25 of highly twisted threads of acetyl cellulose,  
the crepe effect either does not occur at all or else  
only to an extent which is hardly noticeable.  
The highly twisted acetate silk threads do not  
possess therefore, or in any case only to a slight  
30 extent, the property of curling and shrinking in  
contact with warm water.

It has now been found that highly twisted  
threads of acetyl cellulose acquire the property  
35 of producing valuable crepe effects in fabrics  
when treated with water if they contain sub-  
stances which have for water a high affinity.  
Such substances belong to various classes of bodies  
and include, for example, inorganic salts, such  
as calcium chloride or nitrate, or salts of or-  
ganic acids, such as those of lactic acid.

40 The selected substance may be incorporated  
into the threads in various manners. Prefer-  
ably, the selected substance is incorporated in  
the threads prior to the weaving of said threads  
45 into fabrics and prior to the high twisting of the  
yarn. Specifically, the selected substance is in-  
corporated in the yarn by impregnating a skein  
of the yarn with a solution thereof or passing  
the yarn through a solution thereof during the  
50 throwing operation or it is incorporated into the  
spinning solution from which the thread is spun.

In order to obtain crepe effects, acetate silk  
yarns which contain such substances as have been  
mentioned above are highly twisted and made  
to constitute the warp or weft of the fabric. The  
55 fabric thus obtained is thereupon subjected to a

treatment with an aqueous medium. The treat-  
ment can be performed separately or simulta-  
neously with another step in manufacture, as, for  
example, with the treatment in the bath for  
removing the dressing or in the dye bath. 5

## Example I

Ordinary acetate silk threads of 75 deniers  
with 24 individual threads and an arrangement  
of 51 threads to the centimeter are used for the  
warp of a fabric, the weft consisting of acetate  
silk thread containing 10% sodium lactate, twisted  
alternately left and right, of the same standard  
of fineness, having 2800 twists per meter and an  
arrangement of 30 threads to the centimeter. 10  
After weaving, the material is treated in a bath  
with pure water at 85° C. In this way a beau-  
tiful crepe effect similar to crepe-de-Chine is ob-  
tained. 15

## Example II

A skein of 100 denier cellulose acetate thread  
consisting of 32 filaments twisted 2.5 turns per  
inch, is immersed in an aqueous bath containing  
15% by weight of sodium lactate and is allowed  
25 to soak 30 minutes at 120° F. The skein is then  
taken from the bath and whirled for 20 minutes  
in an extractor to remove the major portion of  
the water. The damp, modified thread, contain-  
ing approximately 10% sodium lactate by weight  
30 on the basis of the dry cellulose acetate, and  
optionally a standard yarn dressing composition,  
is given a crepe twist, for instance, 60 turns per  
inch, and is employed as the weft in a fabric con-  
35 taining lowly twisted regenerated cellulose threads  
as the warp. By means of the customary boil-  
off, a retraction of as much as 15% occurs with  
the formation of desirable crepe effects on the  
fabric. 40

## Example III

Approximately 5% by weight of sodium lactate  
is applied to 100 denier cellulose acetate thread  
consisting of 32 filaments twisted 2.5 turns per  
inch during the thread travel to a takeup bobbin  
in a coning, spinning or crepe twisting operation. 45  
The sodium lactate is applied to the thread from  
a 15% aqueous solution of sodium lactate by  
means of a rotating roller, capillary wipers or  
like device in which the upper portion of the  
applying device contacts the thread and the 50  
lower portion contacts the sodium lactate solu-  
tion. After inserting a crepe twist of about 60  
turns per inch and after weaving into a fabric,  
a good quality crepe is secured by submitting  
the fabric to a customary aqueous boil-off.

*Example IV*

Sodium lactate, dissolved in a mixture of acetone and water, is added in sufficient amount to a cellulose acetate spinning solution to yield 5 a spinning solution consisting of 2% sodium lactate and 20% cellulose acetate dissolved in a solvent mixture of 85% acetone and 15% water. The modified spinning solution is converted into a 75 denier thread consisting of 24 10 filaments and the thread is given a crepe twist of about 60 turns per inch. After weaving the crepe twisted thread into fabrics, and after treating the resulting fabrics with an aqueous bath at a temperature of 85° C., a beautiful creped effect similar to crepe-de-Chine is obtained. 15

It is to be understood that the invention is not restricted to the specific details set forth in the examples. For example, by varying the concentration of the sodium lactate solution or time 20 of immersion of the yarn in the solution, a greater or lesser quantity of sodium lactate may be incorporated into the yarn. Satisfactory results have been secured in processing skeins as described in Example II by incorporating 4.5% 25

to 24.3% by weight of sodium lactate on the thread by using an aqueous bath containing 5% to 30% sodium lactate. Also, in the travelling thread method as described in Example III, satisfactory results have been obtained by using 5 15% to 25% aqueous solutions of sodium lactate to incorporate 4.8% to 5.6% by weight of sodium lactate on the dried threads.

This application is a division of application Serial No. 528,240, filed April 6, 1931, now Patent 10 No. 2,107,657.

We claim:

1. A process for producing crepe effects on fabrics which comprises fabricating highly twisted cellulose acetate yarns containing sodium lactate into a fabric, and treating the fabric with an aqueous medium. 15

2. A process for producing crepe effects on fabrics which comprises fabricating highly twisted cellulose acetate yarn containing up to 20 approximately 10% sodium lactate into a fabric and treating the fabric with an aqueous medium. 25

HANS ALTWEGG.  
ARMIN EICHLER.